

Patented June 5, 1923.

## UNITED STATES PATENT OFFICE.

BERTRAND S. SUMMERS, OF PORT HURON, MICHIGAN.

## METHOD OF MAKING PAPER PULP.

Application filed May 26, 1920. Serial No. 384,361.

No Drawing.

To all whom it may concern:

Be it known that I, BERTRAND S. SUMMERS, a citizen of the United States, residing at Port Huron, county of St. Clair, and State of Michigan, have invented certain new and useful Improvements in Methods of Making Paper Pulp, of which the following is a specification.

My invention relates to methods of making paper pulp and especially to a method of treating cereal straws so as to produce therefrom a pulp suitable for the making of high grade paper of uniform quality and free from spots and weaknesses, and has special reference to the preliminary reduction or boiling of such straws to prepare them for final reduction prior to the introduction of the treated material into the beating machine.

Generally speaking, the cereal straws are composed of different parts varying in their chemical composition. They are usually characterized by a thin covering or cuticle and a fibrous portion and joints of more woody nature. Flax has a waxy outer skin containing a pectos fiber surrounding ligneous tissue in the form of a woody tube. These straws, therefore, contain different portions which act differently toward re-agents.

In the treatment of such straws as hitherto practiced it has been customary to subject the straw to a preliminary boiling in an alkaline re-agent, after which boiling the straw has been subjected to a further reduction process prior to transferring the straw to the beating machine. This alkaline treatment, however, effects but very lightly the woody tissue making necessary a very severe subsequent treatment to complete the reduction. If a bi-sulphite of calcium solution of the strength usually used in reducing the wood pulp is used, the bast fiber is very considerably weakened and at the stage when the bast fiber is so weakened the woody portion is imperfectly reduced. It will be seen, therefore, that the action of chemical re-agents on the bast or pectos fiber is notably different than is the effect upon woody or ligneous tissue.

I have discovered that it is possible to so treat the flax straw as to successively reduce the woody portion and then the bast portion without injury to the latter, thus producing a more uniform and cleaner product making possible the production of a

high grade sheet of paper free from spots and of uniform strength.

In practicing my invention I treat the straw in an inclosed vessel with a solution of bi-sulphite of calcium about 3½% strength. This bi-sulphite of calcium is usually about half fixed and half free SO<sub>2</sub>. In lieu, however, of this bi-sulphite of calcium I can use sulphurous acid in which the SO<sub>2</sub> is all free, and obtain practically the same results. The straw is treated with this solution under pressure of 40 to 50 pounds and from 3 to 4 hours, and a bi-sulphite liquor of this strength is added in the ratio of about one-half gallon of said liquor to one pound of straw, sufficient water being added to cover the straw.

After this cook is completed I preferably wash, although the washing operation is not necessary but desirable, and I then subject the straw thus cooked to the action of an alkali for from 3 to 4 hours at 40 to 50 pounds. I usually use a 5% solution of commercial caustic soda, proportionate to the original weight of dry straw. However, other alkali may be used such as alkaline carbonate, alkaline earth hydrates, in fact, any soluble chemical of an alkaline nature. To this alkali may be added a slight amount of oxidizing agent such as bi-oxides or hypo-chlorites, although this addition is not necessary.

After the straw has been cooked in this alkaline bath it is thoroughly washed. At this stage the wood is quite soft and easily disintegrated, and the bast fiber has been considerably dechlorized without decreasing its strength from a paper maker's standpoint.

The composite nature of these straws make it necessary to alternate this treatment, though usually one treatment of an acid followed by the alkali is sufficient. It should be also noted that the first treatment is enhanced by the reducing nature of the acid, it being well known that the bi-sulphite of calcium is a strong reducing agent.

I have also discovered that if other diluted acids are used instead of the bi-sulphite calcium solution in the presence of reducing agents, good effects are obtained and when such treatment is followed by alkaline treatment the straw is reduced to an excellent condition for the final reduction.

The pulp thus prepared is placed in a

suitable vessel and treated with hypo-chlorite calcium solution which has been precipitated out by bicarbonate of soda. Usually 50 or 60 per cent of the hypo-chlorite of calcium is used proportionate to the original weight of straw. This hypo-chlorite is preferably mixed with bicarbonate of soda in dry condition, and water added and thoroughly agitated when the precipitated 10 carbonate of lime is settled and the supernatent liquor is drawn off and introduced on to the mass of straw pulp previously prepared. The pulp is preferably continuously agitated while this final reduction is taking 15 place, which is usually from four to six hours. When the pulp thus prepared is properly obtained, the mass will be found to be of uniform white color and the different compositions making up the straw will 20 be found to have been reduced to practically pure cellulose and all parts so thoroughly

reduced that when the mass is introduced to the paper maker's beating engine it is readily reduced to a pulp from which a good grade of paper is readily obtained. 25

Having now described my invention, what I claim, and desire to secure by Letters Patent is:

1. The herein described process of reducing vegetable straw, which consists in first 30 cooking the straw in a reducing agent having an acid re-action and subsequently cooking it in an oxidizing agent having an alkaline re-action substantially as described.

2. The herein described process of reducing vegetable straw, which consists in first 35 subjecting the said straw to a reducing agent with an acid re-action and subsequently subjecting the said straw to an oxidizing re-agent in an alkaline bath substantially as described. 40

BERTRAND S. SUMMERS.